

106-98

72-27

No. 741,185.

PATENTED OCT. 13, 1903.

J. T. TAYLOR.  
FIREPROOF NAILING BRICK.  
APPLICATION FILED MAY 14, 1903.

NO MODEL.

Fig. 1.



Fig. 2.



Fig. 3.



Schumacher 581112 { 13.13.X

Hummelright 644710 {

Eng 93 - 11187 } Composition (Mar 15)

" 90 - 15784 }

Witnesses:

Ed Kessler.

James L. Morris.

Inventor  
James T. Taylor

James L. Morris

Attest.

## FIREPROOF NAILING-BRICK.

SPECIFICATION forming part of Letters Patent No. 741,185, dated October 18, 1903.

Application filed May 14, 1903. Serial No. 157,170. (No model.)

*To all whom it may concern:*

Be it known that I, JAMES T. TAYLOR, a citizen of the United States, residing at Houston, in the county of Harris and State of Texas, 5 have invented new and useful Improvements in Fireproof Nailing-Brick, of which the following is a specification.

This invention relates to an improved fireproof brick or block to be used as a substitute for the wooden blocks, strips, and plugs now in general use, such wooden pieces being inserted at certain intervals between the course of bricks for the purpose of enabling the interior woodwork to be nailed thereto.

15 The employment of wooden blocks, plugs, strips, or the like is objectionable for many reasons, among which may be mentioned that they frequently split and render the hold of the nail or nails insecure, that they decay 20 under the influence of the atmosphere, that they shrink and draw away from the masonry into which they are built, allowing the same to work loose, and that they increase the danger of destruction of the building in the event 25 of fire.

It is an object of my invention to produce a fireproof brick or block which shall be of a porous character, to enable nails to be driven therein, and which will be free from the objections above set forth.

In order that my invention may be clearly understood, I have illustrated the same in the accompanying drawings, in which—

Figure 1 is a horizontal sectional view of a 35 brick or block constructed according to my invention. Fig. 2 is a cross-section of the same. Fig. 3 is a detailed view showing the strengthening structure.

Proceeding according to my invention I 40 form a composition of Portland cement, cinders, coke, and sand in substantially the proportions, by weight, following: Portland cement, one part; cinders, five parts; coke, one part; sand, two and one-half parts. These 45 ingredients are mixed with a suitable proportion of water to form a plastic mass, and from this mass the bricks or blocks are molded and dried in the usual manner. The coke used is preferably in the form of grains of one-eighth 50 of an inch in size, and the addition of coke in

this form to the composition is for the purpose of rendering the finished product porous in character. I employ coal-cinders—that is, unconsumed particles of coal—as distinguished from ashes or from ordinary furnace refuse, 55 and said cinders are carefully freed from all slag, clinkers, and the like, as these latter ingredients are fused too hard to permit the driving of a nail through the brick and besides would render the same heavy and dense, 60 whereas I aim to produce a light highly-porous brick. The use of cinders and coke crushed to a certain fineness—viz., to about one-eighth of an inch—produces a high degree of porosity and enables the block to 65 yield to the nail, while at the same time rendering it capable of holding the nail as firmly as wood. The sand and cement furnish the material necessary to produce the requisite density and strength. 70

While a brick or block formed of the materials named will ordinarily be strong enough to permit nails to be driven therein without cracking or breaking, I have, nevertheless, found it desirable to absolutely obviate this 75 occurring by strengthening the brick in the manner shown in the drawings—that is to say, I mold in the brick woven wire 1, which is in the form of sheets extending around the sides and end of the bricks at a suitable distance therefrom and of slightly less height than the brick, so that said woven-wire sheets will be entirely embedded in the brick or block. As shown by Fig. 3 these woven-wire sheets are in the form of a rectangle, the 80 opposite sides of which are connected at suitable intervals by diagonal wire braces 2, said braces crossing at the center of the brick 3. Any desired number of these wire braces may 85 be employed. 90

A brick or block constructed according to my invention will be fireproof, will not be deleteriously affected by climatic conditions, while at the same time it will be much stronger than an ordinary wooden block. The 95 addition of the strengthening structure of woven wire prevents all likelihood of the block breaking or splitting when nails are driven into the same.

It will be understood that I can form my 100

741,185

improved block of any desired shape and in different sizes, according to the uses to which it is designed it should be applied.

Having thus fully described my invention, 5 what I claim as new, and desire to secure by Letters Patent, is—

1. A fireproof brick or block composed of Portland cement, coal-cinders, coke and sand.
2. A fireproof brick or block composed of Portland cement, cinders, coke and sand mixed in the proportions by weight, substan-

tially, of one part Portland cement, five parts cinders, one part coke and two and one-half parts sand.

In testimony whereof I have hereunto set 15 my hand in presence of two subscribing witnesses.

JAMES T. TAYLOR.

Witnesses:

E. I. E. RATCLIFFE,

L. S. GREEN.